# EUROPEAN PATENT SPECIFICATION

(11) **EP 0 417 492 B1**
(45) Date of publication and mention of the grant of the patent: **19.04.1995**
(21) Application number: 90115569.7
(22) Date of filing: 14.08.1990
(51) Int. Cl.: B22D 11/128, B22D 11/14

(54) **Vertical continuous casting method and casting apparatus**
Vertikal-Stranggussverfahren und Giesseinrichtung
Coulée continue verticale et appareil de coulée

(30) Priority: 16.08.1989 JP 211067/89; 25.06.1990 JP 164256/90
(43) Date of publication of application: 20.03.1991
(73) Proprietor: DAIDO TOKUSHUKO KABUSHIKI KAISHA, Naka-ku Nagoya-shi Aichi-ken (JP)
(72) Inventor: Morii, Kiyoshi, Kohnan-shi, Aichi-ken (JP); Kumura, Shuzo, Chita-gun, Aichi-ken (JP); Hayakawa, Shyzunori, Tokai-shi, Aichi-ken (JP); Inagaki, Yoshio, Higashiuracho, Chita-gun, Aichi-ken (JP)
(74) Representative: Kraus, Walter, Dr.

(56) References cited:
- WO-A-87/00099
- AU-B- 419 372
- CH-A- 440 569
- FR-A- 1 451 901

## Description

The invention relates to a continuous casting method, wherein a strand formed in a water-cooled mold is drawn down by pairs of rollers vertically therefrom with reducing the strand prior to the solidification point. Furthermore, the invention relates to a vertical continuous casting apparatus comprising a water-cooled mold and its ancillary equipment, reduction means for reducing the strand, drawing drive rolls, and a strand cutter, both positioned downward the water-cooled mold and provided with means for feeding a molten metal to the water-cooled mold. A method and an apparatus of these types are known from WO 87/00099.

Specifically, the invention relates to an improvement of a vertical continuous casting or casting technique of obtaining cast pieces through drawing a strand formed in a water-cooled mold downward without incurvating, and cutting the strand.

Nowadays, a continuous casting process holds an important position in steel casting. However, a horizontal continuous casting process is something problematical in a technical aspect, and hence is only tried in part, and thus what is overwhelming today is a curved and vertical continuous casting. The vertical continuous casting is rather disadvantageous to require a high structure for the equipment, entailing a high cost of equipment. Accordingly, employed prevailingly is the curved continuous casting wherein a strand is incurvated (a water-cooled mold being structured practically so as to provide the curved strand) to extend horizontally, thereby keeping a height of the casting equipment within a certain limit. The strand extending horizontally is rectified to be straight with pinch rolls and cut with a frame cutter into cast pieces.

However, such process comprising curved casting and horizontal rectification is not necessarily preferable for some special steel in respect of quality protection. For example, the rectification operation often causes cracks on the strands of valve steel, high-speed steel and so forth. This kind of steel will have to be subjected to the vertical continuous casting wherein a strand is formed without curvature in the water-cooled mold, drawn straightly downward and cut to cast pieces.

As mentioned in the beginning, vertical continuous casting method and apparatus are known from WO 87/00099. In detail this document describes a method and an apparatus for continuous casting of thin metal products particularly made of steel. According thereto, the internal casting space of the mold is imparted with a substantially spindle-shaped cross-section providing a central portion having a large thickness enabling the introduction of the molten metal stream in normal conditions and having on its sides a reduced thickness corresponding to that of the product to be formed and, into a thickness reducing cage placed immediately at the outlet of the mold, the central portion of the product is progressively flattened until a thickness equal to that of the sides is obtained by exerting throughout the product surface a uniformly distributed pressure so as to continuously straighten the longitudinal walls of the product achieved at the same time as the solidification process at the outlet of the thickness reducing cage.

In the vertical continuous casting, from applying a light reduction to a strand coming out of the water-cooled mold at a position immediately before an unsolidified portion disappears in the interior of the strand, a contraction due to solidification is compensated, and thus, formation of cavities at the center of the strand may be prevented, and center segregation is lessened as well. Thus, cast pieces of better quality can be obtained.

However, in the case of such steel for which the light reduction is effective, a multiple kind is produced relatively in a small quantity in most cases, thus not only a sectional size of the strand varies but also a pertinent drawing speed veries so often, therefore, an optimal position at which the light reduction is to be applied, namely, the point at which the unsolidified portion in the strand disappears may vary one from another.

The object of this invention is to provide a method and apparatus for vertical continuous casting wherein a light reduction is applied to a strand at an optimal position at all times in coping flexibly with casting conditions fluctuating frequently so that the cast pieces of superior quality may be produced.

As regards the method, this object is achieved with a continuous casting method of the type mentioned in the beginning, which is characterized in that a solidification completing point of the strand is determined; that light reduction means comprising pairs of rollers and capable of being variably positioned is positioned just prior to the solidification completing point of the strand; and that light reduction strong enough to compensate for contraction caused by solidification is applied to the strand.

Furthermore, as regards the apparatus, the above object is achieved with a vertical continuous casting apparatus of the type mentioned in the beginning, which is characterized in that light reduction means comprising pairs of rollers is provided variably in position downward the water-cooled mold so as to apply light reduction strong enough to compensate contraction caused by solidification to the strand just prior to the solidification completing point of the strand.

The invention will now be explained in more detail by preferred embodiments thereof with reference to the drawings, wherein:
Fig. 1 is a longitudinal sectional view showing a state of strand interior and a position for light reduction in a continuous casting;
Fig. 2 is a conceptional side view showing a principal part for general construction of a vertical continuous casting apparatus according to this invention;
Fig. 3 to Fig. 5 are detailed drawings exemplifying a mechanism for providing the light reduction means variably in position in the apparatus of Fig. 2; wherein Fig. 3 is a side view, Fig. 4 is a sectional view taken on line I - I of Fig. 3, and Fig. 5 is a sectional view taken on line II - II of fig. 3; and
Fig. 6 is a side view similar to Fig. 3, representing another example of the mechanism for providing the light reduction means variably in position in the apparatus of Fig. 2 likewise.

In a continuous casting method for drawing a strand formed in a water-cooled mold vertically, the method of the present invention comprises, as shown in Fig. 1, positioning light reduction means 4, or pinch rolls representatively, just prior to a solidification completing point of a strand 5A or a point at which an unsolidified portion 52 within a shell 51 disappears, applying light reduction strong enough to compensate contraction caused by solidification of the strand.

In a vertical continuous casting apparatus comprising, as shown in Fig. 2, substantially a water-cooled mold 1 and its ancillary equipment, drawing drive rolls 2 and a strand cutter 3 provided downward the water-cooled mold, and provided with means (not illustrated) for feeding a molten metal to the water-cooled mold, the apparatus of the present invention comprises providing light reduction means 4 variably in position downward the water-cooled mold so as to apply light reduction strong enough to compensate contraction due to solidification to the strand just before the solidification completing point of the strand. A reference character 5B denotes a cast piece obtained from cutting the strand, which will be carried away by a separate device one by one.

The light reduction means and a technique for providing it variably in position are arbitrary, however, devices shown in Fig. 3 to Fig. 5 will be exemplified as typical. The device is constructed such that three pairs of pinch rolls 41a, 41b, 41c are mounted on a frame 42, and the frame 42 is made movable vertically along four pieces of vertical guide columns 43. Each pinch roll is mounted slidably on the frame to advance and retreat by hydraulic cylinders 44a, 44b, 44c fixed on the frame to pinch the strand 5A from opposite sides, driven by motors 45a, 45b, 45c, and is capable of applying a desired light reduction on the strand metal.

Positions of the pinch rolls 41a to c can be changed by worm-jack mechanisms 7 moving vertically from having four pieces of vertical bars 46 on a lower portion of the frame 42 rotated according to rotations of a motor 6 and male screws of the vertical bars engaged with fixed female screws.

Fig. 6 indicates another mode of providing the light reduction means variably in position. In this apparatus, a construction of the light reduction means, namely, the frame and the pinch rolls fitted thereon and other parts is same as the example described above, however, what is different is that a vertical movement of the frame is realized by taking up and delivering a wire 9 laid on pulleys 8a, 8b, 8c, 8d and 8e.

A position of the light reduction means is made variable, adjusted to a solidification completing point fluctuating according to conditions such as steel kind to be subjected to the continuous casting, sectional size of a strand, drawing speed and others, and from carrying out a light reduction at an optimal position, the effect will be enhanced so high.

A determination of the solidification completing point will be made, for example, as follows. That is, since a thickness D of the shell 51 of a strand coming out of the water-cooled mold increases, as a time t passes, in the relation:

$\text{D = k√t}$

a value of k is determined on a techinque wherein a spike is driven, for example, in the strand and then a cast metal is cut to determine whether or not an unsolidified portion is present at the position, and thus the solidification completing point in the strand can be estimated accoding to the above equation.

Recently, there established is a techinque for detecting a solidification completing point by utilizing the phenomenon that a propagation speed of ultrasonic wave varies in solid and liquid. It is therefore preferable that a device for detecting a solid/liquid interface on an ultrasonic wave is added to the light reduction means 4, a solidification completing point in a strand is found to postion the light reduction means in starting the operation, light reduction is thus performed precisely, and when the solidification completing point fluctuates according to changes in steel kind to be subjected to the continuous casting and in casting conditions, the light reduction means is made to follow thereto and the position is modified accordingly.

The strand is drawn by the aforementioned drawing drive rolls, therefore a driving force is not required for the light reduction pinch rolls to have. However, the light reduction pinch rolls will be utilized advantageously for inserting dummy bars into the water-cooled mold when starting the casting operation. The object is attained by providing a driving function to the light reduction pinch rolls, therefore, the aforementioned apparatus is provided with a driving motor.

According to this invention, a light reduction just prior to a solidification completing point in casting a special steel vertically and continuously can be now realized at an optimal position always corresponding to the strand sectional size and changes in casting conditions. Thus, a quality product is ready for securing in meeting severe requirements on quality for the special steel such as prevention of center cavities, lessening of center segregation and so forth.

## Claims

1. A continuous casting method, wherein a strand (5A) formed in a water-cooled mold (1) is drawn down by pairs of rollers vertically therefrom with reducing the strand prior to the solidification point, characterized in that a solidification completing point of the strand is determined; that light reduction means (4) comprising pairs of rollers and capable of being variably positioned is positioned just prior to the solidification completing point of the strand (5A); and that light reduction strong enough to compensate for contraction caused by solidification is applied to the strand (5A).

2. A vertical continuous casting apparatus comprising a water-cooled mold (1) and its ancillary equipment, reduction means for reducing the strand (5A), drawing drive rolls (2), and a strand cutter (3) both positioned downward the water-cooled mold (1), and provided with means for feeding a molten metal to the water-cooled mold (1), characterized in that light reduction means (4) comprising pairs of rollers is provided variably in position downward the water-cooled mold (1) so as to apply light reduction strong enough to compensate contraction caused by solidification to the strand (5A) just prior to the solidification completing point of the strand (5A).

3. A continuous casting apparatus according to claim 2, characterized in that a device for detecting a solid/liquid interface with ultrasonic wave is added to the light reduction means (4) for determining the solidification completing point in the strand so as to position the light reduction means (4) thereto, and when the solidification completing point fluctuates, to vary the position of the light reduction means (4) accordingly thereto.

4. A continuous casting apparatus according to claim 2 or 3, characterized in that the light reduction means (4) is slidable to a frame (42) moving vertically along vertical guide columns (43), and comprises at least a pair of pinch rolls (41a, 41b, 41c) provided so as to pinch the strand (5A) from opposite sides of it by hydraulic cylinders (44a, 44b, 44c).

5. A continuous casting apparatus according to claim 4, characterized in that a drive function is provided to the pinch rolls (41a, 41b, 41c) of the light reduction means (4) to serve as dummy bar pinch rolls at the same time.

## Patentansprüche

1. Stranggießverfahren, worin ein in einer wassergekühlten Form (1) gebildeter Strang (5A) mittels Walzenpaaren vertikal davon nach abwärts gezogen wird, wobei der Strang vor dem Verfestigungspunkt verjüngt, dadurch **gekennzeichnet,** daß ein Verfestigungsvollendungspunkt des Strangs bestimmt wird; daß ein Leichtverjüngungsmittel (4), welches Walzenpaare umfaßt und fähig ist, variabel positioniert zu werden, gerade vor dem Verfestigungsvollendungspunkt des Strangs (5A) positioniert wird; und daß leichte Verjüngung, die stark genug ist, durch die Verfestigung bewirkte Kontraktion zu kompensieren, auf den Strang (5A) angewandt wird.

2. Vertikalstranggießeinrichtung, umfassend eine wassergekühlte Form (1) und ihre Zusatzausrüstung, ein Verjüngungsmittel zum Verjüngen des Strangs (5A), Ziehantriebswalzen (2), und einen Strangschneider (3), die beide abwärts der wassergekühlten Form (1) positioniert sind, und versehen mit einem Mittel zum Zuführen eines geschmolzenen Metalls zu der wassergekühlten Form (1), dadurch **gekennzeichnet,** daß ein Leichtverjüngungsmittel (4), welches Walzenpaare umfaßt, in der Position variabel abwärts der wassergekühlten Form (1) so vorgesehen ist, daß eine leichte Verjüngung, die stark genug ist, um die Kontraktion, welche durch Verfestigung des Strangs (5A) verursacht wird, zu kompensieren, gerade vor dem Verfestigungsvollendungspunkt des Strangs (5A) angewandt wird.

3. Stranggießeinrichtung gemäß Anspruch 2, dadurch **gekennzeichnet,** daß eine Einrichtung zum Detektieren einer Feststoff/Flüssigkeits-Grenzfläche mit Ultraschallwelle zu dem Leichtverjüngungsmittel (4) für das Bestimmen des Verfestigungsvollendungspunkts in dem Strang so hinzugefügt ist, daß das Leichtverjüngungsmittel (4) daran positioniert wird, und wenn der Verfestigungsvollendungspunkt schwankt, daß die Position des Leichtverjüngungsmittels (4) entsprechend dazu variiert wird.

4. Stranggießeinrichtung gemäß Anspruch 2 oder 3, dadurch **gekennzeichnet,** daß das Leichtverjüngungsmittel (4) auf einem Rahmen (42) verschiebbar ist, der sich vertikal längs vertikaler Führungssäulen (43) bewegt, und wenigstens ein Paar Quetschwalzen (41a, 41b, 41c) umfaßt, die so vorgesehen sind, daß sie den Strang (5A) von entgegensetzten Seiten desselben mittels Hydraulikzylindern (44a, 44b, 44c) quetschen.

5. Stranggießeinrichtung gemäß Anspruch 4, dadurch **gekennzeichnet,** daß eine Antriebsfunktion für die Quetschwalzen (41a, 41b, 41c) des Leichtverjüngungsmittels (4) vorgesehen ist, so daß sie gleichzeitig als Blindbarrenquetschwalzen dienen.

## Revendications

1. Procédé de coulée continue, dans lequel un ruban de métal (5A) formé dans un moule refroidi à l'eau (1) est étiré vers le bas par des paires de rouleaux espacées verticalement à partir du moule, avec réduction de section du ruban avant le point de solidification, caractérisé en ce qu'on détermine un point de fin de solidification du ruban ; on dispose des moyens de réduction légère (4), comprenant des paires de rouleaux et dont la position peut être modifiée, juste avant le point de fin de solidification du ruban (5A) ; et on applique au ruban (5A) une légère réduction suffisante pour compenser la contraction résultant de la solidification.

2. Appareil de coulée continue verticale comprenant un moule refroidi à l'eau (1) et son équipement auxiliaire, des moyens de réduction pour réduire la section du ruban de métal (5A), des rouleaux d'entraînement d'étirage (2) et une cisaille de ruban (3), tous placés en aval du moule refroidi à l'eau (1), et comportant des moyens d'amenée d'un métal fondu au moule refroidi à l'eau (1), caractérisé en ce que des moyens de réduction légère (4) comprenant des paires de rouleaux sont prévus à une position variable en aval du moule refroidi à l'eau (1) de façon à appliquer au ruban (5A) une légère réduction suffisamment forte pour compenser la contraction résultant de la solidification, juste avant le point de fin de solidification du ruban (5A).

3. Appareil de coulée continue suivant la revendication 2, caractérisé en ce qu'un dispositif de détection d'une interface solide/liquide au moyen d'ultrasons est ajouté aux moyens de réduction légère (4) pour déterminer le point de fin de solidification du ruban afin de placer les moyens de réduction légère (4) à ce point et, lorsque le point de fin de solidification varie, on modifie la position des moyens de réduction légère (4) conformément à ce point.

4. Appareil de coulée continue suivant la revendication 2 ou 3, caractérisé en ce que les moyens de réduction légère (4) peuvent coulisser dans un cadre (42) déplaçable verticalement le long de montants de guidage verticaux (43), et ils comprennent au moins une paire de rouleaux de pincement (41a,41b,41c) agencés de manière à pincer le ruban de métal (5A) de chaque côté de celui-ci, sous l'action de vérins hydrauliques (44a,44b,44c).

5. Appareil de coulée continue suivant la revendication 4, caractérisé en ce que les rouleaux de pincement (41a,41b,41c) des moyens de réduction légère (4) possèdent une fonction d'entraînement pour servir en même temps de rouleaux de pincement de barres factices.
